

## UNITED STATES PATENT OFFICE

2,105,380

## MANUFACTURE OF ARTIFICIAL SPONGES

Joseph Speijer, Amsterdam, Netherlands

No Drawing. Application January 18, 1936, Serial No. 59,792. In Great Britain April 24, 1935

## 2 Claims. (Cl. 18—48)

It has heretofore been proposed to produce artificial sponges by mixing viscose with fibrous materials and pore-forming substances and subsequently coagulating the viscose.

For this purpose several ways have been suggested using ripened or unripened viscose. In general the use of ripened viscose has the drawback that it yields a product of inferior quality due to the low strength of the product. When using unripened viscose foam-forming substances or anhydrous salts have been employed, which latter may cause an undue coagulation when applied in relatively large quantities.

According to one suggestion a mixture is made from ordinary unripened viscose, prepared from unripened alkali cellulose by adding



together with a proportion of anhydrous sodium sulphate so that the mixture consists of



This mass is placed in a strong coagulating bath, a hot 25% solution of sodium sulphate being a strong coagulator.

According to another suggestion ordinary viscose is mixed with pore-forming fillers. The mass is heated under excess pressure in a regenerating bath. In order to avoid difficulties accruing from the ripeness of the viscose an alkaline regenerating bath is employed.

None of these proposals however pay any attention to the uneven coagulation which will occur even if unripened viscose is used, because it always takes a long time (say 2-4 hours) before the mixing of the mass produces a satisfactory homogeneous product, and during this lapse of time ordinary viscose will start to coagulate even in the presence of sodium sulphate, although sodium sulphate is not a strong coagulator for ordinary unripened viscose when used at room temperature.

According to the present invention unripened viscose is used as an initial material to which an extra quantity of carbon disulphide is added, e. g. 10% of the quantity which has been used for the xanthation, the addition being made immediately before or during the mixing with fibres and pore-forming materials. I will hereinafter use the term "extra CS<sub>2</sub>" to designate this carbon disulphide added after the xanthation treatment, in which CS<sub>2</sub> is employed, e. g. as usual. In this way local coagulation is prevented during the mixing operation, which latter always takes some time. It will be clear that in this

way inner irregularities are prevented and that the product will be thereby maintained more homogeneous.

As a rule crystals of non-acid inorganic salts are to be used as pore-forming fillers. In accordance with my invention it is desirable not to use specifically coagulating salts or acid salts, as has been suggested according to certain prior patent specifications. Specifically coagulating salts are the salts of ammonia and of poly-valent metals, and more especially the acid salts, i. e. the salts with acid reaction such as NaHSO<sub>4</sub> or NaHCO<sub>3</sub> or the like, because of the neutralizing action on the alkali in the viscose. According to the present invention salts are used which in addition to being without any substantial coagulating action on the viscose in the cold, will melt in their own water of crystallization when subsequently heated. For this purpose, salts which melt in their own water of crystallization when heated to about 100° C. (or at any event when heated to not over 150° C.) are preferably used.

Some examples of such salts are:

|                                                        | Melting point      | 25 |
|--------------------------------------------------------|--------------------|----|
|                                                        | degrees centigrade |    |
| Na <sub>2</sub> SO <sub>4</sub> . 10 aq.               | 32.4               |    |
| Na <sub>3</sub> PO <sub>4</sub> . 12 aq.               | 73.4               |    |
| Na <sub>2</sub> HPO <sub>4</sub> . 12 aq.              | 34.6               |    |
| Na <sub>2</sub> CO <sub>3</sub> . 10 aq.               | 34.0               | 30 |
| Na <sub>2</sub> B <sub>4</sub> O <sub>7</sub> . 10 aq. | 75.0               |    |

In regenerating the mixture one proceeds preferably in such a way that the outside of the "cake" to be regenerated (in a mold, or not) obtains a certain degree of solidity as soon as possible, e. g. by bringing the mass into a very warm environment. In this operation, the molds are preferably brought into a heated chamber (e. g. a chamber heated directly or indirectly by steam, to about 100° C. or somewhat higher), which heat may be continued for 3 to 15 hours, 6 hours being suitable. Here heat may serve as the regenerating medium. The masses (in molds or not) can then be placed into a heated waterbath in order to dissolve and remove the pore-forming substances. It is also possible to place the masses in a setting bath substantially consisting of a watery solution of sodium sulphide and sodium sulphate. This solution may serve as the regenerating bath, sodium sulphide also acting as the desulphurizing agent.

It is usually advisable not to subject the mixture of viscose, etc., and salts, to a too high temperature because of the fact that temperatures

higher than a 150° are liable to cause deterioration of the cellulose. Accordingly, it is advisable to bring the filled molds into a room with a temperature of about 100° C.

5 In order to elucidate my invention the following example is given:—

The viscose can be prepared, for example by impregnating 100 parts of cellulose with an excess of 18% NaOH solution, and then (after letting stand for 2 to 5 hours if desired) pressing or centrifuging the mixture down to about 430 parts. This presscake (alkali cellulose) will contain about 100 parts of cellulose, about 60 parts of NaOH and about 270 parts of water. 10 to 40 parts of CS<sub>2</sub> are allowed to act upon the comminuted alkali cellulose, in the usual manner, to xanthate the same. The xanthated material is then dissolved in such amounts of water and caustic soda as to give a viscose containing preferably about 6-8% of cellulose, and about 5-7% of NaOH. Or the xanthate can be dissolved in water alone if desired. To the freshly prepared viscose is added (per 100 parts of cellulose contained therein) about 10-30 parts of fibres (e. g., 15 flock of cotton, flax, hemp, etc.) and about 3-4 parts of CS<sub>2</sub> (i. e. the "extra CS<sub>2</sub>" mentioned above). This latter quantity of CS<sub>2</sub> is preferably added while thoroughly mixing the fibres with the viscose. Then to the mixture of viscose, fibres 20 and extra carbon bisulphide (i. e., the 3-4 parts added after the xanthation and dissolution have been carried out) is at once added one or several of the crystalline salts mentioned above, e. g., a quantity of 300-800 parts by weight for every 25 100 parts by weight of viscose.

If the crystals are small (e. g., passing a 20 mesh screen and retained on a 50 mesh screen) this will produce small fine pores in the resulting sponge, while large crystals with an average 30 diameter of  $\frac{1}{8}$  to  $\frac{1}{2}$  inch will produce larger pores in the sponge.

The mass obtained in this way is introduced 35 into molds and thereupon the mass is subjected to a very warm atmosphere (for, say, 6 hours), or this can be done after a period (say 2-4 hours) 40 of rest in order to allow the mass to become as homogeneous as possible. In consideration of

the fact that the regeneration of the cellulose takes place quicker at a higher temperature, it will be evident that temperatures above 100° C. are desired to shorten the reaction. The heating of the molds is then carried out as indicated above, and also the treatment with the setting bath.

5 After regeneration, the washing, desulphurization (if needed as a separate step), bleaching and such like operations can be carried out as usual.

It will be evident to the expert that many modifications may be carried out lying within the scope of the present invention. For example, the proportions and the sequence of the 15 additions may be varied within considerable limits, e. g., the extra carbon disulphide may be added before the fibers are added, or it may be added simultaneously with the crystals.

I claim:—

20 1. A process of manufacturing artificial sponges from viscose which comprises adding extra carbon disulphide and pore-forming material solids to unripened viscose, the extra carbon disulphide being in addition to that used in the xanthation of the cellulose, said extra carbon disulphide being in amount capable of preventing premature coagulation of the viscose by the pore-forming solids, and regenerating the cellulose of the viscose, while the pore-forming solid 25 remains chemically undecomposed.

2. In a process of making artificial sponge the steps of adding to unripened viscose, about 3% to 4% of carbon disulphide, based on the cellulose content of the said viscose, and adding an 30 amount of crystals, containing water of crystallization, which is substantially larger than the amount of cellulose, said crystals being such as can melt in their own water of crystallization at temperatures not above 150° C., and being crystals which do not exert a substantial coagulation 35 action on viscose in the cold, making the mixture uniform and then subjecting the viscose to coagulation by heat, and heating the mass sufficiently to cause the crystals to melt, and wash- 40 45 the sponge so produced.

JOSEPH SPEIJER.